

# United States Patent

[11] 3,615,378

[72] Inventors **Howard B. Bomberger, Jr.**  
**Canfield;**  
**Stanley R. Seagle, Warren; Ronald R.**  
**Seeley, Canfield, all of Ohio**  
[21] Appl. No. **764,585**  
[22] Filed **Oct. 2, 1968**  
[45] Patented **Oct. 26, 1971**  
[73] Assignee **Reactive Metals, Inc.**

|           |         |                    |            |
|-----------|---------|--------------------|------------|
| 2,721,137 | 10/1955 | Pitler.....        | 75/175.5   |
| 2,754,204 | 7/1956  | Jaffee et al.....  | 75/175.5   |
| 2,798,806 | 7/1957  | Jaffee et al.....  | 75/175.5   |
| 2,804,409 | 8/1957  | Kessler et al..... | 75/175.5 X |
| 2,857,269 | 10/1958 | Vordahl .....      | 75/175.5   |
| 2,880,089 | 3/1959  | Vordahl .....      | 75/175.5   |
| 2,892,706 | 6/1959  | Jaffee et al.....  | 75/175.5   |
| 2,968,586 | 1/1961  | Vordahl .....      | 75/175.5 X |
| 3,405,016 | 10/1968 | Jaffee et al.....  | 75/175.5 X |

[54] **METASTABLE BETA TITANIUM-BASE ALLOY**  
**8 Claims, 2 Drawing Figs.**

Primary Examiner—Charles N. Lovell  
Attorney—Walter P. Wood

[52] U.S. Cl..... 75/175.5  
[51] Int. Cl..... C22c 15/00  
[50] Field of Search..... 75/175.5,  
148/32, 133

[56] **References Cited**  
UNITED STATES PATENTS  
2,596,485 5/1952 Jaffee et al..... 75/175.5

**ABSTRACT:** A metastable beta titanium-base alloy in which beta stability is achieved by optimum addition of beta-eutectoid element (iron, manganese, chromium and/or cobalt). Also included are beta-isomorphous elements (vanadium and/or molybdenum), aluminum, and optionally one or both the neutral elements (tin and zirconium). Alloy is readily formable at room temperatures and can be heat-treated to high tensile strength.

PATENTED OCT 26 1971

3,615,378



FIG. 1.



FIG. 2.

INVENTORS.  
HOWARD B. BOMBERGER JR.,  
STANLEY R. SEAGLE and  
RONALD R. SEELEY  
By Walter P. Wood  
Attorney

## METASTABLE BETA TITANIUM-BASE ALLOY

This invention relates to an improved high-strength metastable beta titanium-base alloy.

Titanium-base alloys used for structural purposes in the aircraft and aerospace industries should possess several important characteristics. The alloy should be produced readily as a mill product, such as sheet, strip, plate, bar, billet, tubing or wire, by melting, forging, rolling or other commercial metalworking processes. Preferably final production and fabrication of sheet, strip, tubing and wire are performed at room temperature for reasons of efficiency and economy and to attain a desirable surface finish and properties. In its annealed or softened state the alloy should have sufficient ductility (10 percent minimum elongation in 2 inches) to allow considerable forming at room temperature. It should be possible to bend a sheet of the alloy to a radius less than twice its thickness without breaking the sheet. The least radius to which a sheet can be bent is referred to as its "minimum bend radius" (MBR) and is usually expressed as a ratio of radius-to-thickness. The alloy should respond to heat treatment and achieve heat-treated yield strengths greater than 160 K.s.i. with useful toughness and ductility (4 percent minimum elongation in 2 inches), which properties it should retain after prolonged exposure to temperatures up to 600° F. under allowable design stresses. The alloy also should have high strength-to-weight ratios which are needed in weight-critical structures.

It is well known that titanium metal may exist as an alpha phase, a beta phase, or an alpha-beta structure which is a mixture of the two phases. At room temperature the pure metal assumes the alpha phase, which has a closely packed hexagonal crystalline structure. On heating above the beta transus temperature (about 1,625° F.), the pure metal assumes the beta phase, which has a body-centered cubic crystalline structure. The beta phase can be retained wholly or in part at room temperature by adding to titanium certain alloying elements known as beta stabilizers. These may be either beta-eutectoid elements, such as iron, manganese, chromium, cobalt or nickel, or beta-isomorphous elements, such as vanadium, molybdenum, columbium or tantalum. Usually the alpha phase has greater mechanical strength than the beta phase, but less ductility. The alpha-beta structure represents a compromise which affords both the strength and ductility needed for many applications.

Most previous attempts to meet the requirements hereinbefore stated have involved the use of alpha-beta alloys, which usually are processed at high temperatures with little cold reduction possible between annealing and cleaning treatments. High-temperature metalworking often necessitates an expensive surface cleaning operation of the product after it has been hot-worked or formed. These alloys are limited to moderate yield strength ranges of 120 to 150 K.s.i. with limited ductility and toughness.

An object of our invention is to provide a metastable all-beta titanium-base alloy which possesses the desirable characteristics hereinbefore listed.

A further object is to provide an alloy which has these characteristics and can be produced with conventional mill equipment and is sufficiently ductile to be cold-worked and finished at room temperature, yet can be simply heat treated to medium and high strengths.

A further object is to provide an alloy of the foregoing characteristics in which we control the average valence electron density (VED) to a critical range (about 4.15 to 4.30).

In the drawing:

FIG. 1 is a typical phase diagram of a titanium-beta-eutectoid element system; and

FIG. 2 is a graph illustrating how we determine the theoretical maximum content of beta-eutectoid elements in our alloy.

Our alloy contains one or more of the beta-eutectoid elements iron, manganese, chromium or cobalt. These elements have advantages for stabilizing the beta phase of titanium alloys, since they are compatible with the melting process (no master alloys required), they are relatively lightweight compared with the beta-isomorphous elements, and they are

strong beta stabilizers. However, if they are added to a titanium alloy in excessive quantities, compounds form and ductility is lost. Preferably we include in our alloy beta-eutectoid elements near the maximum quantities that do not form compounds. We look to the phase diagrams to determine the content we can safely include.

As FIG. 1 shows, some known percentage of a beta-eutectoid element added to titanium forms a eutectoid at some known temperature, indicated at point *b*. The percentage and temperature of course are different for each beta-eutectoid element, but all follow a similar pattern. Line *a-b* represents the boundary between the beta phase and the beta-plus-compound. We extrapolate line *a-b* to 752° F. to determine the theoretical maximum content of the element which can be included at this temperature without forming a compound, indicated at point *c*. Similarly we extrapolate the line to room temperature (approximately 50° to 100° F.) to determine the maximum at room temperature, indicated at point *d*.

FIG. 2 shows the extrapolation for the five beta-eutectoid elements iron, manganese, chromium, cobalt and nickel. The extrapolated curves for the first four reach room temperature at atomic percentages of the element ranging from about 3.5 to 8.5, but the extrapolated curve for nickel never reaches room temperature. Hence we may use any of the first four elements, but not nickel, as beta stabilizers in our alloy. We limit the content of beta-eutectoid element in our alloy to the maximum established by extrapolation of the curves to room temperature. In this manner we arrive at the following content for each element when used individually:

## Atomic Percent

|    |           |            |
|----|-----------|------------|
| 35 | Iron      | Up to 4.5% |
|    | Manganese | Up to 6.0% |
|    | Chromium  | Up to 8.5% |
|    | Cobalt    | Up to 3.5% |

We may use these elements in combination, but the total must not exceed the maximum of any element used individually. Thus the limiting combined total in atomic percentages is given by the equation:

$$\%Fe+4.5/6(\% Mn)+4.5/8.5(\% Cr)+4.5/3.5(\% Co)=4.5\%$$

Even though the beta-eutectoid elements are highly effective for stabilizing the beta phase, we cannot include them in our alloy in a sufficiently high content that by themselves they retain an all-beta structure at room temperature. Accordingly we add one or more beta-isomorphous elements in the following approximate proportions:

## Atomic Percent

|    |            |          |
|----|------------|----------|
| 55 | Vanadium   | 2 to 16% |
|    | Molybdenum | 1 to 6%  |
|    | Columbium  | 3 to 23% |
|    | Tantalum   | 3 to 21% |

The beta-isomorphous elements thus supplement the beta-eutectoid elements in stabilizing the beta phase in our alloy. We presently prefer vanadium and molybdenum because of their lower cost and greater efficiency as beta stabilizers.

Our alloy also contains aluminum in proportions of about 1.75 to 7 atomic percent. We use aluminum as a strengthening agent. Usually aluminum is an alpha promoter and inhibits retention of the beta phase at room temperature. We overcome this effect of aluminum in our alloy by our inclusion of large quantities of beta-eutectoid and beta-isomorphous elements already described.

Our alloy also may contain at least one of the neutral elements tin and zirconium in the following approximate proportions:

## Atomic Percent

|           |          |
|-----------|----------|
| Tin       | Up to 3% |
| Zirconium | Up to 3% |

The preferred composition of our alloy is within the following approximate range (excluding incidental impurities):

## Atomic Percent

|                      |             |
|----------------------|-------------|
| Fe, Mn, Cr and/or Co | 2 to 7%     |
| V                    | 4 to 9%     |
| Mo                   | 1.5 to 3%   |
| Al                   | 3.5 to 7%   |
| Sn and/or Zr         | 1.5 to 2.5% |
| Ti                   | Balance     |

The neutral elements improve the ductility of our alloy and retard formation of an undesirable brittle omega phase.

We have found that a necessary condition for a titanium-base alloy to retain an all-beta structure at room temperature is that it have an average valence electron density (VED) above 4, usually at least 4.15. To calculate the average VED of an alloy, the atomic percent of each element is multiplied by the number of its valence electrons, and the sum of these products is divided by 100. Titanium itself has 4 valence electrons, as have the neutral alloying elements zirconium and tin. Aluminum has 3 valence electrons, and as already mentioned is an alpha stabilizer, which retards formation of the beta phase. The beta-isomorphous elements vanadium, columbium and tantalum have 5 valence electrons, while molybdenum has 6. The beta-eutectoid elements which we can use have valence electrons as follows:

|           |   |
|-----------|---|
| Iron      | 8 |
| Manganese | 7 |
| Chromium  | 6 |
| COBalt    | 9 |

The calculation of the VED of a titanium-base alloy is given by the following equation using atomic percentages:

$$VED = 0.04(\%Ti + \%Zr + \%N) + 0.07(\%Mn) + 0.06(\%Cr + \%Mo) + 0.08(\%Fe) + 0.09(\%Co) + 0.05(\%V + \%Cb + \%Ta) - 0.03(\%Al)$$

Our alloy has a VED of 4.15 to 4.35, which we regard as critical as demonstrated hereinafter by actual examples.

15 Specific nominal compositions which we have found advantageous are as follows in atomic percents:

|                                  |
|----------------------------------|
| 2.5% Fe or 3.5% Mn or 5.5% Cr or |
| 2.0% Co                          |
| V-7.5%                           |
| Mo-2%                            |
| Al-5.5%                          |
| Ti-Balance                       |

20 Preferably we add to any of these latter compositions tin and/or zirconium in amounts of approximately 1.5 to 2.5 percent of the alloy.

30 In the tables which follow, we show the properties of a number of specific alloys. The first three alloys listed in table I fall outside our invention, while the others are within. Alloy 1 has a VED below our critical range and its MBR is much too high. Alloys 2 and 3 have VED at or above the upper limit of our critical range. While they meet bend requirements, aging produces no significant increase in their hardness or tensile strength.

TABLE I.—PROPERTIES OF METASTABLE BETA-TITANIUM ALLOY SHEET

| Alloy No. | Composition, atomic percent                            | VED  | Heat treatment                                    | Hardness, Rockwell A | UTS, Ks.i. | YS, Ks.i. | El, percent | MBR, R/T |
|-----------|--------------------------------------------------------|------|---------------------------------------------------|----------------------|------------|-----------|-------------|----------|
| 1.....    | Ti-2.1, Mo-1.9, V-1.8, Fe.....                         | 4.13 | 1450 F.-12 min.-AC.....                           | 74                   | 165        | 165       | 0           | >        |
| 2.....    | Ti-3.1, Mo-7.9, V-7.2, Fe.....                         | 4.43 | 1450 F.-12 min.-AC.....<br>+900 F.-24 hr.-AC..... | 67                   | 189        | 136       | 22          | 0.7      |
| 3.....    | Ti-3.2, Mo-8.1, V-6.5, Mn-1.7, Sn.....                 | 4.35 | 1460 F.-10 min.-AC.....<br>+900 F.-8 hr.-AC.....  | 65                   | 127        | 123       | 16          | 1.0      |
| 4.....    | Ti-2.0, Mo-7.6, V-4.4, Mn-6.4, Al.....                 | 4.20 | 1550 F.-12 min.-AC.....<br>+900 F.-8 hr.-AC.....  | 63                   | 113        | 108       | 9           | 0.8      |
| 5.....    | Ti-3.1, Mo-7.6, V-2.8, Fe-5.4, Al.....                 | 4.19 | 1560 F.-12 min.-AC.....<br>+900 F.-8 hr.-AC.....  | 66                   | 113        | 108       | 10          | 1.0      |
| 6.....    | Ti-3.1, Mo-7.7, V-5.6, Cr-5.4, Al.....                 | 4.21 | 1560 F.-12 min.-AC.....<br>+900 F.-8 hr.-AC.....  | 64                   | 188        | 191       | 4           |          |
| 7.....    | Ti-3.1, Mo-7.6, V-3.5, Mn-5.4, Al.....                 | 4.19 | 1550 F.-12 min.-AC.....<br>+900 F.-4 hr.-AC.....  | 72                   | 191        | 184       | 4           | 1.0      |
| 8.....    | Ti-2.1, Mo-7.8, V-4.5, Fe-3.8, Zr-5.5, Al.....         | 4.24 | 1400 F.-12 min.-AC.....<br>+1000 F.-8 hr.-AC..... | 66                   | 69         |           |             |          |
| 9.....    | Ti-2.1, Mo-7.9, V-1.8, Fe-3.7, Mn-2.5, Sn-5.6, Al..... | 4.26 | 1560 F.-12 min.-AC.....<br>+1000 F.-8 hr.-AC..... | 63                   |            |           |             |          |
| 10.....   | Ti-2.0, Mo-7.5, V-5.5, Cr-6.2, Al.....                 | 4.16 | 1600 F.-7 min.-AC.....<br>+950 F.-8 hr.-AC.....   | 120                  | 115        | 15        | 0.9         |          |
| 11.....   | Ti-1.7, Mo-7.6, V-3.5, Mn-5.3, Al.....                 | 4.17 | 1600 F.-7 min.-AC.....<br>+950 F.-8 hr.-AC.....   | 181                  | 163        | 8         |             |          |
| 12.....   | Ti-6.4, Mo-2.8, Mn-1.7, Sn-4.8, Al.....                | 4.17 | 1450 F.-10 min.-AC.....<br>+900 F.-8 hr.-AC.....  | 125                  | 121        | 10        | 0.7         |          |
| 13.....   | Ti-3.1, Mo-2.0, V-1.8, Fe-3.6, Mn-3.3, Zr-5.6, Al..... | 4.21 | 1560 F.-12 min.-AC.....<br>+1000 F.-8 hr.-AC..... | 194                  | 186        | 5         |             |          |
| 14.....   | Ti-3.1, Mo-7.6, V-2.0, Co-5.5, Al.....                 | 4.19 | 1550 F.-12 min.-AC.....<br>+900 F.-8 hr.-AC.....  | 65                   | 72         |           |             |          |

TABLE II.—PROPERTIES OF HIGH STRENGTH TITANIUM ALLOYS

| Composition, atomic percent                    | Density, lb./cu. in. | Heat treatment <sup>1</sup> | UTS, Ks.i. | YS, Ks.i. | El, percent | MBR, R/T |
|------------------------------------------------|----------------------|-----------------------------|------------|-----------|-------------|----------|
| Ti-3.1, Mo-7.7, V-3.6, Mn-5.4, Al.....         | 0.170                | ST                          | 126        | 122       | 15.8        | 1.0      |
| Ti-3.1, Mo-7.8, V-3.6, Mn-2.1, Zr-5.5, Al..... | 0.172                | STA                         | 198        | 184       | 5.8         |          |
| Ti-3.0, Mo-7.6, V-4.7, Cr-5.4, Al.....         | 0.171                | STA                         | 134        | 132       | 12.0        | 1.0      |
| Ti-2.0, Mo-7.6, V-5.5, Cr-5.4, Al.....         | 0.169                | STA                         | 200        | 187       | 7.5         |          |
| Ti-3.0, Mo-7.6, V-3.5, Mn-7.2, Al.....         | 0.170                | STA                         | 196        | 179       | 7.0         |          |
| Ti-1.5, Mo-7.7, V-4.5, Mn-1.6, Sn-5.4, Al..... | 0.171                | STA                         | 121        | 116       | 14.8        | 0.9      |
| Ti-2.0, Mo-7.6, V-2.7, Fe-5.5, Al.....         | 0.170                | STA                         | 132        | 127       | 8.5         |          |
|                                                |                      | STA                         | 203        | 185       | 6.5         |          |
|                                                |                      | STA                         | 129        | 124       | 13.0        | 1.1      |
|                                                |                      | STA                         | 204        | 189       | 6.9         |          |
|                                                |                      | STA                         | 121        | 113       | 13.5        | 1.7      |
|                                                |                      | STA                         | 185        | 173       | 7.2         |          |

<sup>1</sup> ST=Solution-Treated; STA=Solution-Treated and Aged.

TABLE III.—STABILITY OF HIGH STRENGTH TITANIUM ALLOY

| Composition, atomic percent               | Before creep  |              |                | After creep            |               |              |                |
|-------------------------------------------|---------------|--------------|----------------|------------------------|---------------|--------------|----------------|
|                                           | UTS,<br>Ks.i. | YS,<br>Ks.i. | EI,<br>percent | Creep exposure         | UTS,<br>Ks.i. | YS,<br>Ks.i. | EI,<br>percent |
| Ti-3.1, Mo-7.7, V-3.6, Mn-5.4, Al         | 198           | 184          | 5.8            | 600 F.-115 Ks.i.-96 hr | 197           | 189          | 6.8            |
| Ti-3.1, Mo-7.8, V-3.6, Mn-2.1, Zr-5.6, Al | 206           | 192          | 4.5            | 600 F.-115 Ks.i.-96 hr | 199           | 190          | 6.0            |
| Ti-3.0, Mo-7.6, V-4.7, Cr-5.4, Al         | 195           | 179          | 7.0            | 600 F.-115 Ks.i.-96 hr | 201           | 192          | 4.5            |
| Ti-2.0, Mo-7.6, V-5.5, Cr-5.4, Al         | 174           | 158          | 9.0            | 600 F.-85 Ks.i.-96 hr  | 177           | 160          | 0.5            |
| Ti-3.0, Mo-7.6, V-3.5, Mn-7.2, Al         | 202           | 182          | 7.5            | 600 F.-85 Ks.i.-96 hr  | 196           | 171          | 4.3            |
| Ti-3.0, Mo-7.6, V-3.5, Mn-7.2, Al         | 202           | 182          | 7.5            | 500 F.-85 Ks.i.-96 hr  | 194           | 172          | 6.5            |
| Ti-1.5, Mo-7.7, V-4.5, Mn-1.8, Sn-5.4, Al | 206           | 190          | 7.6            | 550 F.-85 Ks.i.-96 hr  | 198           | 179          | 6.5            |

We claim:

1. A metastable beta titanium-base alloy which consists essentially of:
  - a. at least one beta-eutectoid element selected from the group which consists of iron, manganese, chromium and cobalt in a maximum content determined by the equation:  

$$\%Fe+4.5/6(\%Mn)+4.5/8.5(\%Cr)+4.5/3.5(\%Co)=4.5\%$$
  - b. 4 to 9 percent vanadium,
  - c. 1.5 to 3 percent molybdenum,
  - d. 3.5 to 7 percent aluminum,
  - e. balance titanium and incidental impurities,
 the foregoing quantities being in terms of atomic percentages, said alloy having an average valence electron density of about 4.15 to 4.35.
2. An alloy as defined in claim 1 containing in addition at least one neutral element selected from the group which consists of tin and zirconium in amounts up to approximately 3 percent of the alloy.
3. An alloy as defined in claim 1 in which the beta-eutectoid element is selected from the group which consists of Fe in the

amount of approximately 2.5 percent of the alloy, Mn in the amount of approximately 3.5 percent of the alloy, Cr in the amount of approximately 5.5 percent of the alloy, and Co in the amount of approximately 2.0 percent of the alloy, the remainder of the composition being approximately as follows:

V 7.5%

Mo 2%

Al 5.5%

Ti Balance.

4. An alloy as defined in claim 3 in which the beta-eutectoid element is iron.

5. An alloy as defined in claim 3 in which the beta-eutectoid element is manganese.

6. An alloy as defined in claim 3 in which the beta-eutectoid element is chromium.

7. An alloy as defined in claim 3 in which the beta-eutectoid element is cobalt.

8. An alloy as defined in claim 3 containing in addition at least one neutral element selected from the group consisting of tin and zirconium in amounts of approximately 1.5 to 2.5 percent of the alloy.

UNITED STATES PATENT OFFICE  
CERTIFICATE OF CORRECTION

Patent No. 3,615,378 Dated October 26, 1971  
Inventor(s) Howard B. Bomberger, Jr., et al.

It is certified that error appears in the above-identified patent and that said Letters Patent are hereby corrected as shown below:

Column 3, line 34, "ZR" should read -- Zr --; same line "N" should read -- Sn --; line 35, the minus sign (-) preceding "0.03 (% Al)" should read -- + --. Column 4, Table I, under "MBRM R/T" first line ">" should read -- >25 --.

Signed and sealed this 21st day of November 1972.

(SEAL)

Attest:

EDWARD M. FLETCHER, JR.  
Attesting Officer

ROBERT GOTTSCHALK  
Commissioner of Patents